# EUROPEAN PATENT SPECIFICATION

(11) **EP 1 772 528 B1**
(45) Date of publication and mention of the grant of the patent: **30.01.2013**
(21) Application number: 04745513.4
(22) Date of filing: 02.06.2004
(51) Int. Cl.: C22C 14/00, C22F 1/18, C22F 1/00

(54) **TITANIUM ALLOY AND METHOD OF MANUFACTURING TITANIUM ALLOY MATERIAL**
TITANLEGIERUNG UND VERFAHREN ZUR HERSTELLUNG VON TITANLEGIERUNGSMATERIAL
ALLIAGE DE TITANE ET PROCEDE DE FABRICATION DE MATERIAU EN ALLIAGE DE TITANE

(43) Date of publication of application: 11.04.2007
(73) Proprietor: Nippon Steel & Sumitomo Metal Corporation, Tokyo 100-8071 (JP)
(72) Inventor: KURODA, Atsuhiko c/o Sumitomo Metals, Joetsu-shi, Niigata 9420011 (JP)
(74) Representative: Benson, John Everett
(86) International application number: PCT/JP2004/007614
(87) International publication number: WO 2005/118898

(56) References cited:
- JP-A- 4 301 044
- JP-A- 5 117 791
- JP-A- 62 284 060
- JP-A- 2004 183 079
- JP-A- 2004 183 079
- US-A- 4 299 626
- US-A- 5 980 655

## Description

The present invention relates to titanium alloys in use in chemical industry members such as machine structure members and heat exchanger members and consumer goods members such as golf clubs, and a method for manufacturing titanium alloy materials. The present invention particularly relates to titanium alloys with an excellent cold workability and superplasticity characteristics, and a method for manufacturing the titanium alloy materials.

Heat exchangers are instruments capable of transmitting thermal energy between different fluids. The heat exchangers are used in, for example, air conditioners, refrigerators, air preheating equipment of burners, radiators in automobiles, parts for the chemical industry, parts for seawater and the like. In particular, heat exchangers made of titanium are used in fields requiring excellent corrosion resistance such as in the chemical industry or in salt water. In order to reduce the size of heat exchangers, it is necessary to increase the strength of the parts being used and that is why titanium alloy which are light and strong are used as a material for such heat exchangers.

A Ti-6Al-4V alloy has been widely used as the heat exchanger material due to its excellent superplasticity characteristics as described in, for example, Non-patent document 1. However, this alloy has poor cold workability. For example, when thin plates are manufactured by cold rolling the Ti-6A1-4V alloy plate which is wrapped around a coil, there is a drawback that the number of intermediate annealing needs to be increased.

Non-patent document 2 shows that a Ti-9V-2Mo-3Al alloy is a titanium alloy which has an excellent cold workability and also an excellent superplasticity workability. However, this alloy contains Mo as an essential element, which results in a high cost of raw materials. Also, because of a high melting point of Mo, there is a higher incidence of unmelted portions or solidification segregation in melting.

Patent document 1 describes a titanium alloy with excellent superplasticity workability containing, by mass %, A1 of 5.5 to 6.5%, V of 3.5 to 4.5%, O of 0.2% or less, Fe of 0.15 to 3.0%, Cr of 0.15 to 3.0% and Mo of 0.85 to 3.15%, in which Fe, Cr and Mo are within a range represented by a specific equation and an average grain diameter of an α crystal is 6µm or less. This alloy can be said to be superior to the Ti-6AI-4V alloy in the superplasticity workability, but the cold workability is not considered. Namely, this alloy has a high content of A1 which is 5.5% or more, which results in high deformation resistance in the cold rolling and a high possibility of cracks occurring in the edges of a plate if this alloy is subjected to cold rolling process at a cross-section reduction rate of 50%.

Patent document 2 describes a titanium alloy with excellent workability which contains, by mass %, A1 of 3.0 to 5.0%, V of 2.1 to 3.7%, Mo of 0.85 to 3.15%, O of 0.15% or less, and further one or more elements of Fe, Cr, Ni and Co, in which the content of these elements is in a range represented by a specific equation. There is also described a manufacturing method of a titanium alloy material in a specific hot rolling condition, and a superplastic processing method of the titanium alloy material in the specific heat treatment condition. However, since this alloy contains Mo, there will be the same problem with the alloy described in Non-patent document 2.

Patent document 1: Japanese Examined Patent Publication No. 1996-19502B
Patent document 2: Japanese Examined Patent Publication No.1996-23053B
Non-patent document 1: N. Furushiro and three other persons, Titanium' 80, 1980, pp. 993-998, published by Metallurgical Society of AIME
Non-patent document 2: T. Oka and 2 other persons, "What is being studied about titanium materials in Japan?", pp. 58-60, edited on Dec. 1, 1989 by The Iron and Steel Institute of Japan
US-A-5980 655 relates to ballistic armour Ti-6A1-4V alloys with high oxygen content. US 2, 804, 409 describes titanium alloy products and particularly thin section products.

An object of the present invention is to provide titanium alloys with the excellent cold workability and the superplasticity characteristics and a method for manufacturing the titanium alloy materials. Means adapted to solve the problem

The present invention was accomplished as a result of repeated research made by the present inventors based on a Ti-3A1-2.5V alloy which is said to have the excellent cold workability.

The present invention is characterized by titanium alloys as shown in (1) below, and a method for manufacturing a titanium alloy material as shown in (2) below.

(1) A cold rolled titanium alloy plate consisting of, by mass %, A1 of 2.0 to 4.0%, V of 4.0 to 9.0%, Zr of not more than 2.0%, Sn of not more than 3.0%, and optionally further containing one or more elements selected from Fe of 0.20 to 1.0%, Cr of 0.01 to 1.0%, Cu of 0.01 to 1.0% and Ni of 0.01 to 1.0%, and the balance being Ti and impurities, wherein Veq obtained by the following equation (1) is in a range of 4.0 to 9.5: $Veq = V + 1.9 ⁢ Cr + 3.75 ⁢ Fe$
where a symbol on a right side of the equation (1) means a content of each element, by mass %, wherein the cold rolled titanium alloy plate is obtainable by subjecting the titanium alloy to cold working at a cross-section reduction rate of 40% or more.

(2) A method for manufacturing cold rolled titanium alloy plate is characterized in that the titanium alloy described in the above (1) is subjected to cold working at a cross-section reduction rate of 40% or more.

### Effect of the Invention

A titanium alloy of the present invention has a sufficient cold workability as well as the excellent superplasticity characteristics. Therefore, it is possible to easily produce a coil by the cold rolling, and a material for a super-plastic application, having a uniform distribution in a plate thickness, can be manufactured. Therefore, it is possible to easily produce thin plates made of titanium alloy at a low cost, allowing for the expansion of an application field for the titanium alloy thin plates. Best mode for carrying out the invention

First, chemical compositions in the titanium alloy of the present invention and the reasons for the limitation will be described. "%" in each component means "mass %" in the following explanation.

### Al: 2.0 to 4.0%

Al is an element that plays a very important role in increasing the strength of the titanium alloy. Al is also an effective element for stabilizing the α phase of the titanium alloy The superplasticity characteristics are exhibited in a temperature range in which the ratio of the a phase and the β phase is approximately 50/50. If the content of A1 is low, this temperature range is narrowed, which results in difficulties obtaining stable superplasticity characteristics. The content ofAl needs to be 2.0% or more so as to obtain the superplasticity characteristics in a wider temperature range. However, the cold workability reduces as the content ofAl increases. In particular, if a titanium alloy in which the content of Al exceeds 4.0% is subjected to the cold working at a cross-section reduction rate of about 50%, the edge cracks occur in the edges of the plate. Therefore, the content of A1 is limited to 2.0 to 4.0%.

### V: 4.0 to 9.0%

V is an effective element for stabilizing the β phase of titanium alloys, and has an effect of increasing the ratio of the β phase in a temperature range of about 800 to 850 °C. In particular, if the content of V is 4.0% or more, the temperature range in which the ratio of the α phase and the B phase is approximately 50/50 can be increased. However, if the content of V exceeds 9.0%, oxidation resistance characteristics of the titanium alloy material are deteriorated. This is because an oxide of V has a sublimation property, so that a scale generated on the surface of the alloy is not dense but has a high permeability of oxygen if the titanium alloy in which the content of V exceeds 9.0% is exposed to a high temperature. Therefore, cracks occur more easily on the surface of the alloy, and a high temperature ductility is decreased. Accordingly, the content of V is limited to 4.0 to 9.0%.

### Zr: 0 to 2.0%

Zr is an element that may not be optionally added. If Zr is added, it contributes to strengthen the titanium alloy due to a solid solution strengthening effect thereof. If a titanium alloy containing Zr is exposed to the high temperature, a strong Zr oxide is formed on the surface thereof to suppress oxidation inside the alloy, so that a generation of the cracks can be prevented in a deformation of the titanium alloy at the high temperature. Therefore, elongation of the titanium alloy is increased at the high temperature, and the superplasticity characteristics are improved. These effects are largely exhibited in 0.5% or more. However, Zr is an expensive element, and the oxidation suppression effect described above is saturated if the content of Zr exceeds 2.0%, leading to a cost increase. Therefore, if Zr is contained, the content is preferably limited to 2.0% or less.

### Sn: 0 to 3.0%

Sn is also an element that may not be necessarily added. Although Sn does not contributes to stabilize the α phase or the β phase, it is an element that contributes to strengthen the titanium alloy To obtain such effect of Sn, the content is preferably 0.2% or more. However, if the content of Sn exceeds 3.0%, a low melting point region is formed in solidification process, and the cracks occur from this region as a starting point. Therefore, if Sn is contained, the content is preferably 3.0% or less.

Certain titanium alloys of the present invention have the chemical compositions described above, the balance being Ti and impurities. Other alloys of the invention contain one or more elements selected from Fe of 0.20 to 1.0%, Cr of 0.01 to 1.0%, Cu of 0.01 to 1.0% and Ni of 0.01 to 1.0% as substitute for a part of Ti. This is based on the following reasons.

Fe and Cr are elements contained, as impurities, in a titanium sponge which is a titanium raw material, or in an aluminum-vanadium alloy which is an additional material. Therefore, Fe of less than 0.20% and Cr of less than 0.01% are contained in the titanium alloy even if these elements are not positively added. These elements are β-phase stabilizing elements having the same effect as V, but they are cheaper than V. Accordingly, cost reduction can be realized by positively adding these elements, so that it is desirable to contain Fe of 0.20% or more and Cr of 0.01% or more. However, Fe and Cr are eutectoid type elements forming an intermetallic compound in the titanium alloy. If the Fe and Cr contents exceed 1.0% each, there will be embrittlement caused by excessive precipitation of the intermetallic compound.

Cu and Ni are β stabilizing elements in the same manner as V, and are effective to increase the ratio of the B phase in a temperature range of 800 to 850 °C. These elements are cheaper than V, and can be added as an alternative element to V It is desirable to use Cu at 0.01% or more and Ni at 0.01% or more in order to obtain this effect. However, an intermetallic compound is formed and cold workability is lowered if Cu or Ni exceed 1.0% each, because Cu and Ni are eutectoid type elements for titanium.

Accordingly, if one or more elements of these are contained in the titanium alloy of the present invention, the content is limited to Cr of 0.01 to 1.0%, Cu of 0.01 to 1.0% and Ni of 0.01 to 1.0%, and the value of Veq is restricted as follows: $Veq ⁢ \left(=V+1.9⁢Cr+3.75⁢Fe\right) : 4.0 to 9.5$

Veq is an index to exhibit the stability of the β phase in the titanium alloy, and is represented by the following equation (1): $Veq = V + 1.9 ⁢ Cr + 3.75 ⁢ Fe$
where the symbol of an element on the right side of the equation (1) means the content of that element.

If the Veq is less than 4.0, the ratio of the β phase is lowered in a temperature range of 800 to 850 °C, and the superplasticity characteristics are hardly exhibited in this temperature range. However, if the Veq exceeds 9.5, the ratio of the α phase is lowed, the superplasticity characteristics deteriorate in a temperature range of 800 to 850 °C and the specific gravity of the alloy itself increases. Accordingly, if Fe and/or Cr are contained to the titanium alloy of the present invention, it is necessary to limit Veq in a range of 4.0 to 9.5.

O (oxygen), C (carbon), N (nitrogen) and H (hydrogen) are major impurities contained in the titanium alloy of the present invention. O is an impurity contained in the titanium sponge and a raw material of V, while C and N are impurities contained in the titanium sponge. Also, H is an impurity which is absorbed from an atmosphere in heating or absorbed in an acid pickling process. Impurities are preferably as low as possible in a range where O is 0.2% or less, C is 0.01% or less, N is 0.01% or less, and H is 0.01% or less.

Next, a method for manufacturing titanium alloy plate of the present invention will be explained. An ingot is prepared by an ordinary melting method such as VAR and is subjected to hot bloom forging or hot rolling so as to form a slab, after which hot rolling is conducted to prepare a hot coil, followed by the cold rolling to a target plate thickness and annealing to provide the titanium alloy material. The cold rolling is a step that largely influences product characteristics, and a titanium alloy material with the excellent superplasticity characteristics at the high temperature can be obtained particularly by the cold working (cold rolling) at the cross-section reduction rate of 40% or more. This is based on the following reasons.

When the cross-section reduction rate is increased in the cold rolling, a crystal grain diameter in the titanium alloy, particularly a grain diameter of a pro-eutectoid α phase is decreased. Then, if the grain diameter in the titanium alloy is decreased, elongation is increased upon superplastic deformation at the high temperature, thereby the titanium alloy material with the excellent superplasticity characteristics at the high temperature is exhibited. As described above, when the cross-section reduction rate is increased in the cold rolling, the elongation upon superplastic deformation at the high temperature is sharply increased up to the cross-section reduction rate of about 40%, and less change is observed in a region of 40% or more.

Therefore, in the method for manufacturing the titanium alloy materials of the preset invention, the cold working is performed at the cross-section reduction rate of 40% or more. Although there is no particular upper limit in the cross-section reduction rate, when the cold rolling is performed at a cross-section reduction rate of exceeding 80%, the edge cracks occur in the edges of the plate. Accordingly, it is desirable in the cold working to limit the cross-section reduction rate in 80% or less. However, if the intermediate annealing is conducted for the purpose of recovering the ductility of materials, the cold working may be performed in a condition that the cross-section reduction rate exceeds 80%.

The cross-section reduction rate is obtained by the following equation (a). $Cross - section reduction rate \left(%\right) = \left\{\left(cross-section area before working cross-section area after working\right)/cross-section area before working\right\} \times 100$

### Example 1

Using an arc melting furnace of plasma, a button ingot with a width of 50 mm, a thickness of 15 mm and a longitude of 80 mm was prepared. After the button ingot was heated at 850 °C, it was subjected to hot rolling to prepare a hot-rolled plate with a thickness of 5 mm. After this hot-rolled plate was annealed at 750 °C for ten minutes, an oxide scale was removed by shot blast and acid pickling, and the surface was further machined to a thickness of 4mm by machining so as to prepare a material for the cold rolling. This material was subjected to the cold rolling to prepare a cold-rolled plate with a thickness of 2 mm. At this time, as an evaluation of cold-rolling property, presence of cracks in the edges on the surface of the cold-rolled plate was performed by visual observation.

A plate with no cracks in the cold rolling was subjected to a heat treatment in an argon atmosphere at 700 °C for 30 minutes, followed by cold rolling to a thickness of 1.5 mm, and again subjected to the heat treatment in the argon atmosphere at 700 °C for 30 minutes to provide a test specimen. From this test specimen, a plate type test piece with a thickness of 1.5 mm and a width of 12.5 mm in a parallel part was obtained so that the longitudinal direction of the test piece was in parallel to the rolling direction. The distance between gauge marks of this tensile test piece was set to be 20mm, and a tensile test was conducted at a test temperature of 800 °C and a tensile speed of 9 mm/min., so as to measure elongation at fracture.

Table 1 shows chemical compositions of the cold-rolled plate, evaluations of cold rolling property and elongation at fracture.

**[Table 1]**

| No. | Chemical composition (mass %, the balance being Ti and impurities) | | | | | | | | | Cold rolling property evaluation | Elongation at fracture | | Remarks |
|---|---|---|---|---|---|---|---|---|---|---|---|---|---|
| | Al | V | Zr | Sn | Fe | Cr | Cu | Ni | Veq | | Elongation (%) | Evaluation | |
| 1 | 1.58* | 5.08 | - | - | - | - | - | - | 5.5 | ○ | 180 | × | Comparative example |
| 2 | 2.05 | 4.96 | - | - | - | - | - | - | 5.4 | ○ | 320 | ○ | Example of the present invention |
| 3 | 3.00 | 4.98 | - | - | - | - | - | - | 5.6 | ○ | 440 | ○ | Example of the present invention |
| 4 | 3.96 | 4.90 | - | - | - | - | - | - | 5.5 | ○ | 470 | ○ | Example of the present invention |
| 5 | 4.20* | 4.94 | - | - | 0.24* | - | - | - | 5.8 | × | - | - | Comparative example |
| 6 | 3.01 | 3.50* | - | - | - | - | - | - | 4.1 | ○ | 160 | × | Comparative example |
| 7 | 3.05 | 4 12 | - | - | - | - | - | - | 4.8 | ○ | 295 | ○ | Example of the present invention |
| 8 | 3.00 | 7.02 | - | - | - | - | - | - | 7.7 | ○ | 400 | ○ | Example of the present invention |
| 9 | 2.98 | 8.88 | - | - | - | - | - | - | 9.4 | ○ | 320 | ○ | Example of the present invention |
| 10 | 3.01 | 5.05 | - | - | 0.50* | - | - | - | 6.9 | ○ | 355 | ○ | Comparative Example |
| 11 | 3.03 | 4.98 | - | - | 0.98* | - | - | - | 8.7 | ○ | 275 | ○ | Comparative Example |
| 12 | 3.02 | 5.11 | - | - | 1.20* | - | - | - | 9.6* | ○ | 150 | × | Comparative example |
| 13 | 2.99 | 4.97 | - | - | - | 0.485 | - | - | 6.3 | ○ | 335 | ○ | Example of the present invention |
| 14 | 2.97 | 4.96 | - | - | - | 0.95 | - | - | 7.2 | ○ | 300 | ○ | Example of the present invention |
| 15 | 2.99 | 5.00 | - | - | - | 2.21* | - | - | 9.6* | × | - | - | Comparative example |
| 16 | 3.02 | 5.01 | - | - | 0.50* | 1.15* | - | - | 9.1 | × | - | - | Comparative example |
| 17 | 3.04 | 4.90 | - | - | 0.88* | 1.01* | - | - | 10.2* | ○ | 125 | × | Comparative example |
| 18 | 3.03 | 4.98 | 0.51 | - | - | - | - | - | 5.5 | ○ | 310 | ○ | Example of the present invention |
| 19 | 3.00 | 5.03 | 0.95 | - | - | - | - | - | 5.6 | ○ | 335 | ○ | Example of the present invention |
| 20 | 3.05 | 4.98 | 1.88 | - | - | - | - | - | 5.4 | ○ | 340 | ○ | Example of the present invention |
| 21 | 3.00 | 5.01 | - | - | 0.98* | - | - | - | 8.7 | ○ | 275 | ○ | Comparative Example |
| 22 | 3.03 | 5.05 | - | - | - | - | 0.05 | - | 5.6 | ○ | 420 | ○ | Example of the present invention |
| 23 | 3.01 | 5.02 | - | - | - | - | 0.98 | - | 5.6 | ○ | 435 | ○ | Example of the present invention |
| 24 | 3.02 | 4.98 | - | - | - | - | 1.13* | - | 5.6 | × | - | - | Comparative example |
| 25 | 2.99 | 5.01 | - | - | - | - | - | 0.08 | 5.7 | ○ | 410 | ○ | Example of the present invention |
| 26 | 3.00 | 5.03 | - | - | - | - | - | 0.75 | 5.7 | ○ | 405 | ○ | Example of the present invention |
| 27 | 2.99 | 5.05 | - | - | - | - | - | 1.28* | 5.6 | × | - | - | Comparative example |
| 28 | 3.02 | 4.97 | - | 0.15 | - | - | - | - | 5.6 | ○ | 425 | ○ | Example of the present invention |
| 29 | 3.03 | 5.02 | - | 0.88 | - | - | - | - | 5.7 | ○ | 430 | ○ | Example of the present invention |
| 30 | 3.00 | 5.04 | - | 1.55 | - | - | - | - | 5.7 | ○ | 440 | ○ | Example of the present invention |
| 31 | 2.99 | 4.99 | - | 2.85 | - | - | - | - | 5.6 | ○ | 400 | ○ | Example of the present invention |
| 32 | 3.02 | 5.01 | - | 3.10* | - | - | - | - | 5.6 | × | - | - | Comparative example |
| 33 | 3.01 | 6.51 | - | - | 0.90* | - | - | - | 9.9* | ○ | 170 | × | Comparative example |
| 34 | 321 | 7.02 | - | - | 0.51* | 0.45 | - | - | 9.8* | ○ | 165 | × | Comparative example |
| 35 | 311 | 7.55 | - | - | - | 0.95 | | - | 10.0* | ○ | 135 | × | Comparative example |

| | | | | | | | | | | | | | |
|---|---|---|---|---|---|---|---|---|---|---|---|---|---|
| (1) [*] means outside of the range specified in the present invention (2) [-] in the chemical composition means an impurity level, in which Fe is less than 0.20% and other than Fe is less than 0.01%. (3) Examples with [×] in the cold rolling property had no tensile test conducted. | | | | | | | | | | | | | |

In the cold rolling property evaluation, a plate with no cracks is indicated as [○] and a plate with cracks is indicated as [×] when a cold-rolled plate with a thickness of 2 mm was prepared. Also, in the elongation at fracture, a plate of exceeding 200% in elongation at fracture is indicated as [○], and a plate of 200% or less in elongation at fracture is indicated as [×] when a tensile test was conducted at 800 °C.

As shown in Table 1, alloys satisfying the chemical compositions specified in the present invention are capable of being cold rolled to obtain an excellent superplastic elongation.

### Example 2

A material for cold rolling containing Al of 3.0%, V of 5.0% and the balance being Ti and impurities was prepared with a thickness of 4 mm in the same manner with Example 1.

The material for cold rolling was subjected to a cold rolling in different cross-section reduction rates to prepare cold-rolled plates with thicknesses of 3.5 mm, 3.0 mm, 2.5 mm, 2.0 mm and 1.5 mm. After these cold-rolled plates were subjected to the heat treatment in the argon atmosphere at 700 °C for 30 minutes, a plate type test piece with a thickness of 1.0 mm and a width of 12.5 mm in a parallel part was obtained so that the longitudinal direction of the test piece was in parallel with the rolling direction. The distance between the gauge marks in this tensile test piece was set to 20 mm, and the tensile test was conducted at the test temperature of 800 °C and a tensile speed of 9 mm/min., so as to measure the elongation at fracture.

Further, in order to examine the influence of a cross-section reduction rate to the superplasticity characteristics in the cold rolling after the intermediate annealing, the cold-rolled plate with a thickness of 2.0 mm was subjected to the heat treatment in the argon atmosphere at 700 °C for 30 minutes, followed by the cold rolling to a thickness of 1.5 mm or 1.0 mm, and again subjected to the hot treatment in the argon atmosphere at 700 °C for 30 minutes so as to prepare a test specimen. From this test specimen, the plate type test piece with the thickness of 1.0 mm and the width of 12.5mm in the parallel part was obtained, and the same tensile test as described above was conducted to measure the elongation at fracture. Table 2 shows the cross-section reduction rate and the elongations at fracture.

**[Table 2]**

| No. | Before intermediate annealing | | After intermediate annealing | | Elongation rate at fracture (%) |
|---|---|---|---|---|---|
| | Plate thickness after cold rolling (mm) | Cross-section reduction rate (%) | Plate thickness after cold rolling (mm) | Cross-section reduction rate (%) | |
| 36 | 3.50 | 12.5* | - | - | 210 |
| 37 | 3.02 | 24.5* | - | - | 240 |
| 38 | 2.47 | 38.3* | - | - | 360 |
| 39 | 1.99 | 50.3 | - | - | 470 |
| 40 | 1.51 | 62.3 | - | - | 485 |
| 41 | 2.02 | 49.5 | 1.52 | 24.8 | 440 |
| 42 | 2.03 | 49.3 | 1.05 | 48.3 | 425 |

| | | | | | |
|---|---|---|---|---|---|
| *Outside the scope of invention | | | | | |

As shown in Table 2, since all the examples are within a range of the chemical compositions specified in the present invention, the elongation at fracture exceeds 200% and the excellent superplasticity characteristics have been obtained. In particular, the elongation at fracture is increased in accordance with the increase of the cross-section reduction rate, and there is almost no change in the elongation at fracture under a condition that the cross-section reduction rate is 40% or more. Also, from the results of No. 39 and No. 40, it is understood that an excellent elongation at fracture is observed if the cross-section reduction rate before the intermediate annealing is 40% or more, even though the cold rolling rate after the intermediate annealing is low.

### Industrial Applicability

The titanium alloy of the present invention has the sufficient cold workability as well as the excellent superplasticity characteristics. Accordingly, it is possible to easily prepare the coil by the cold rolling, and also to manufacture a material for a super-plastic application having a uniform distribution in a plate thickness. Therefore, the titanium alloy thin plates can be easily manufactured at a low cost, allowing the expansion of the application field for the titanium alloy thin plates.

## Claims

1. A cold rolled titanium alloy plate consisting of, by mass %, Al of 2.0 to 4.0%, V of 4.0 to 9.0%, Zr of not more than 2.0%, Sn of not more than 3.0% and optionally further containing one or more elements selected from Fe of 0.20 to 1.0%, Cr of 0.01 to 1.0%, Cu of 0.01 to 1.0% and Ni of 0.01 to 1.0% and the balance being Ti and impurities, wherein Veq obtained by the following equation (1) is in a range of 4.0 to 9.5: $Veq = V + 1.9 ⁢ Cr + 3.75 ⁢ Fe$
wherein the symbol of an element on the right side of the equation (1) means the content of the element by mass %,
wherein the cold rolled titanium alloy plate is obtainable by subjecting the titanium alloy to cold working at a cross-section reduction rate of 40% or more.

2. A cold rolled titanium alloy plate according to claim 1 containing at least 0.2% Sn.

3. A method for manufacturing a cold rolled titanium alloy plate according to claim 1 or claim 2, which comprises subjecting a titanium alloy having the composition set out in claim 1 or claim 2 to a cold working at a cross-section reduction rate of 40% or more.

## Patentansprüche

1. Kaltgewalzte Titanlegierungsplatte, bestehend aus, in Massenprozent, Al 2,0 bis 4,0%, V 4,0 bis 9,0%, Zr nicht mehr als 2,0%, Sn nicht mehr als 3,0%, und gegebenenfalls außerdem enthaltend ein oder mehr Elemente, ausgewählt aus Fe mit 0,20 bis 1,0%, Cr mit 0,01 bis 1,0%, Cu mit 0,01 bis 1,0% und Ni mit 0,01 bis 1,0% und wobei der Rest Ti und Verunreinigungen ist, wobei Veq, das durch die folgende Gleichung (1) erhalten wird, in einem Bereich von 4,0 bis 9,5 liegt: $Veq = V + 1 , 9 ⁢ Cr + 3 , 75 ⁢ Fe$
wobei das Symbol eines Elementes auf der rechten Seite der Gleichung (1) den Gehalt des Elements in Massenprozent bedeutet,
wobei die kaltgewalzte Titanlegierungsplatte erhalten wird, indem die Titanlegierung einem Kaltwalzen bei einer Querschnittsverringerungsrate von 40% oder mehr unterworfen wird.

2. Kaltgewalzte Titanlegierungsplatte gemäß Anspruch 1, die wenigstens 0,2% Sn enthält.

3. Verfahren zur Herstellung einer kaltgewalzten Titanlegierungsplatte gemäß Anspruch 1 oder Anspruch 2, das Unterwerfen einer Titanlegierung, die die in Anspruch 1 oder Anspruch 2 angegebene Zusammensetzung hat, einer Kaltbearbeitung bei einer Querschnittsverringerungsrate von 40% oder mehr umfasst.

## Revendications

1. Plaque en alliage de titane laminée à froid constituée, en % en masse, de 2,0 à 4,0 % d'Al, de 4,0 à 9,0 % de V, d'au plus 2,0 % de Zr, d'au plus 3,0 % de Sn et contenant éventuellement en outre un ou plusieurs éléments choisis parmi 0,20 à 1,0 % de Fe, 0,01 à 1,0 % de Cr, 0,01 à 1,0 % de Cu et 0,01 à 1,0 % de Ni, le reste étant du Ti et des impuretés, dans laquelle la valeur Veq, obtenue par l'équation (1) suivante, est située dans la plage allant de 4,0 à 9,5 : $Veq = V + 1 , 9 ⁢ Cr + 3 , 75 ⁢ Fe$
dans laquelle le symbole d'un élément du côté droit de l'équation (1) signifie la teneur en l'élément, en % en masse,
laquelle plaque en alliage de titane laminée à froid peut être obtenue par l'opération consistant à soumettre l'alliage de titane à un usinage à froid avec un taux de réduction de section transversale de 40 % ou plus.

2. Plaque en alliage de titane laminée à froid selon la revendication 1 contenant au moins 0,2 % de Sn.

3. Procédé pour fabriquer une plaque en alliage de titane laminée à froid selon la revendication 1 ou la revendication 2, qui comprend l'opération consistant à soumettre un alliage de titane ayant la composition indiquée dans la revendication 1 ou la revendication 2 à un usinage à froid avec un taux de réduction de section transversale de 40 % ou plus.
